

H. DICKE.

PROCESS OF REFINING AND AGGLOMERATING ORES AND THE LIKE.

APPLICATION FILED MAY 25, 1904.

986,271.

Patented Mar. 7, 1911.

Fig. 2.



Fig. 1.



Inventor

Hugo Dicke

By his atty

Penruie Goldborough

Witnesses:

Chas. J. O'Neill

J. E. Hutchinson Jr.

# UNITED STATES PATENT OFFICE.

HUGO DICKE, OF FRANKFORT-ON-THE-MAIN, GERMANY, ASSIGNOR TO JACOB EDUARD GOLDSCHMID, OF FRANKFORT-ON-THE-MAIN, GERMANY.

## PROCESS OF REFINING AND AGGLOMERATING ORES AND THE LIKE.

986,271.

Specification of Letters Patent. Patented Mar. 7, 1911.

Application filed May 25, 1904. Serial No. 209,794.

To all whom it may concern:

Be it known that I, HUGO DICKE, head engineer, residing at 14 Neue Mainzerstrasse, Frankfort-on-the-Main, Germany, have in-

5 vanted new and useful Improvements in Processes of Refining and Agglomerating Ores and the Like, of which the following is a specification.

The present invention relates primarily 10 to the treatment of those ores which can only be smelted with difficulty, first on account of their physical condition and secondly on account of the injurious foreign substances which they contain. To this class 15 belong more particularly the friable iron ores.

According to the present invention ores 20 of the aforesaid class are treated in a revolving furnace in such manner that their objectionable physical and chemical characteristics are rendered innocuous, and so that there will pass out of the furnace from the dusty material (containing injurious substances) which was charged thereinto a refined product of lumpy consistency, which approximates the general formula of  $Fe_3O_4$ . This is a result which cannot be obtained 25 with an ordinary revolving furnace, for the reason that in the latter the method of firing 30 is unsuitable. The practice has generally been to employ coal dust as fuel. It has also been proposed to pass the gaseous products of combustion from an ordinary furnace grate through such furnaces for the purpose of drying the ores and of causing them 35 to fuse together. But this is only possible in a few simple cases and the addition of certain materials or even of coal dust for the purpose of facilitating the fusibility of 40 the ores has been necessary. Such a method has great drawbacks and is not adapted for extended use.

According to my invention the revolving furnace is heated by a water gas flame 45 whereby entirely new results are achieved and many fields of use are opened up. By the employment of a water gas flame, not only can all the results heretofore obtained be effected in a more simple and certain 50 manner, but it is also possible (owing to the peculiar formation of the flame) to so perform the operations in the furnace that oxidation or reduction and fusion, shall take place at will.

55 The essential advantage of the water gas

flame over the processes hitherto used is the possibility of regulating its nature according to the nature of the material undergoing treatment.

In the practice of my invention, I have ascertained that what is called a neutral water gas flame viz. a flame out of a mixture to which exactly the chemical equivalent of air is added will reduce ores of the formula  $Fe_2O_3$  to  $Fe_3O_4$ ; and this will even keep on, if the flame is slightly oxidizing.

The flame is to be regulated so that no flame appears outside the end of the furnace. Hereto the oxygen evolved by the reduction is to be taken into account. The products so obtained are ready for treatment in blast furnaces or any equivalent apparatus.

The possibility of regulating the character of the flame allows of the treatment of other products also as for instance the waste products of sulfuric acid works, of anilin works, and of the copper metallurgical processes. These substances (known as pyritis cinder, and blue-billy) are extremely difficult to treat in the blast furnace because owing to their friability they render the column of the furnace charge too dense. Moreover they often contain a high percentage of substances such as arsenic or sulfur which have an injurious effect upon the quality of the pig iron. The presence of zinc moreover may lead to the formation of a crust of zinc sponge which not only injures the quality of the iron but also prejudicially affects the actual working of the blast furnace. In the manufacture of lead or copper, a similar unfavorable effect is produced by the presence of arsenic, antimony and sulfur.

The working of the furnace may be so regulated as to enable three zones to be distinguished therein, there being effected in the highest portion of the furnace, drying and preliminary heating; in the middle portion, oxidation and fusion; and in the lower portion, reduction and distillation. Of course these operations may also be separately carried out in different furnaces. It is thus rendered possible to remove the water from an ore, to roast the ore, to melt out admixtures, or to remove them by reduction, oxidation or distillation, in one continuous operation.

The accompanying drawings illustrate a furnace of the kind referred to, adapted more

particularly for the treatment of "purple ore" (blue-billy), or the residues of roasted pyrites (pyritis cinder), or the like, in which sulfur, zinc, and lead are required to be removed from the iron before the latter is smelted in the blast furnace or before its introduction into the open hearth furnace.

Figure 1 represents a longitudinal sectional view of said furnace. Fig. 2 represents a section taken on a plane indicated by the line 2-2 of Fig. 1.

*a* is the revolving drum which is lined with an acid or basic refractory material, and into which the ore is charged at its upper end through the chute *b*. The ore first passes through the drying zone *c* and then enters the oxidizing zone *d*. Here the sulfur, arsenic, zinc and the like are oxidized and also volatilized, while the residual ore begins to fuse together in lumps and nodules. Any zinc which has not yet been volatilized as zinc oxid passes into the reducing zone *e* where it is volatilized as metallic zinc. Any lead that may be present is also reduced and melted here, and runs off through the annular passage *f* (which is provided with apertures *g*) into molds *h*. The ore passes out from the lower end of the furnace not only in a physical condition adapted for blast furnace treatment, but also purified, and in a lower stage of oxidation.

For the purpose of keeping the oxidizing and reducing zones effectually separated from each other, the gas and air are preferably admitted wholly or partially at different places. The wide pipe *m* serves for the admission of the water gas which can become ignited at the mouth of this pipe even without any previous admixture of air, while the quantity of air which is necessary for complete combustion or the excess air requisite for oxidation, is admitted through the air pipe *n* at a place situated farther back.

It is obvious that, by regulating the quantities of gas and air admitted, as well as by the manner in which and the place whereat the gas and air are mixed together, every possible desirable result can be obtained. This adaptability of the furnace constitutes its chief value, since it enables materials to be treated which have no homogeneous or uniform composition.

The furnace is to be used in the same manner whether iron ores, copper ores or by-products containing a high percentage of copper, are to be treated, the lead, zinc, sulfur, arsenic and antimony being similarly separated. These separated products may be recovered for use according to the special economic conditions in each case. As will be seen by the drawing the waste gases may be cooled by means of a water spray so that

the volatile metallic oxides are precipitated in the form of mud and may be removed in that condition.

65

What I claim is:

1. The process of agglomerating fine iron ores or residues, which consists in subjecting the same to a temperature which shall cause the particles thereof, due to the impurities contained therein, to fuse sufficiently to become semiplastic and sticky, and agitating, by rolling the mass, when in the semiplastic state.

2. The process of desulfurizing and agglomerating fine iron ores or residues, which consists in eliminating the sulfur by means of an oxidizing atmosphere at a temperature best suited for that purpose, and then moving the mass into a temperature which shall cause the particles thereof, due to the impurities contained therein, to fuse sufficiently to become semiplastic and sticky, and agitating the mass by revolving it about a horizontal or inclined axis.

75

3. The process of agglomerating fine iron ores or residues, which consists in passing the same through a rotating kiln having a region in which the degree of temperature shall cause the particles thereof, due to the impurities contained therein, to fuse sufficiently to become semiplastic and sticky.

80

4. The process of desulfurizing and agglomerating fine iron ores or residues, which consists in passing the same through a rotating kiln, in one part of which it shall be exposed to an oxidizing atmosphere at a temperature best suited for its desulfurization, and in another part of which it shall be exposed to a temperature which shall cause the particles thereof, due to the impurities contained therein, to fuse sufficiently to become semiplastic and sticky.

85

5. The method of treating friable ores and the like preliminary to their reduction in a blast furnace or the like, by a water gas flame in a revolving furnace.

90

6. The method of treating friable iron ores preliminary to their reduction in a blast furnace or the like, by a regulable water gas flame in a revolving furnace producing a lumpy product of the formula  $Fe_3O_4$ .

100

7. The method of agglomerating pulverulent iron ores or the like, which consists in effecting the dissociation of  $Fe_2O_3$  therein into  $Fe_3O_4$  by the action of a heating flame, and nodulizing, by rolling the mass.

115

In testimony whereof, I have signed my name to this specification, in the presence of two subscribing witnesses.

HUGO DICKE.

Witnesses:

JEAN GRUND,  
CARL GRUND.